

Oct. 19, 1943.

R. E. T. HAFF ET AL

2,331,974

ORNAMENTATION

Filed Oct. 11, 1941

*Fig. 1*



*Fig. 5* *Fig. 6*

*Fig. 3*

*Fig. 2*



*Fig. 7* *Fig. 8* *Fig. 9*

*Fig. 4*



Raymond E. T. Haff  
John C. Creadick  
Thomas F. Banigan

INVENTORS  
BY *Paul B. Selle*  
ATTORNEY

## UNITED STATES PATENT OFFICE

2,331,974

## ORNAMENTATION

Raymond E. T. Haff, Greeneville, Del., and John Conlyn Creadick and Thomas F. Banigan, Kenmore, N. Y., assignors to E. I. du Pont de Nemours & Company, Wilmington, Del., a corporation of Delaware

Application October 11, 1941, Serial No. 414,590

8 Claims. (Cl. 41—17)

This invention relates to ornamentation, especially to rendering bottles more attractive by means of shrinkable, cellulosic bands or secondary closures which resemble gold foil, and it comprehends the discovery that a regenerated cellulose band having a blended outer mica particle and yellow coloring matter-containing layer and an inner titanium dioxide particle-containing layer effectively simulates a metallic gold appearance.

Custom has long required that bottles of many types of alcoholic liquors, particularly wines, have the upper part of the neck, and the closure, encased in a very thin metal capsule or a wrapping of metal foil. This practice has also been adopted for a great deal of the bottled non-alcoholic beverages for the primary purpose of sales appeal. This type (metal foil) of secondary closure has many disadvantages, inter alia, poor fit resulting in an unattractive appearance, lack of adhesion which allows it to slip off the bottle neck before the time of wilful removal, and complete opaqueness requiring that sections be cut out if visual inspection of the underlying material is to be made.

Shrinkable, tube-shaped, regenerated cellulose bands have been used as secondary closures for bottles for some years, because they act effectively to secure easily displaceable primary closures, as deterrents against tampering, aid in positioning revenue stamps, etc. (see U. S. A. Patent No. 1,647,489 to Webster). Since these bands can be colored and printed upon, they may contribute to the decorative appearance of the unit.

To seal and/or decorate a bottle, the shrinkable band in gel (hydrated) form is placed over the bottle top (the primary closure, such as stopper or screw cap, being in place) and allowed to dry. The water evaporating from the band causes it to shrink and fit into very firm engagement with the underlying structure.

The conventional details of band manufacture are disclosed in U. S. A. Patent No. 2,161,561 (and 1,647,489) to Dalton, and since the processing is analogous to that employed with cellulose sheet (see U. S. A. Patents No. 1,548,864, 1,601,289, and 2,123,883), reference is made to such prior art for conventional details in the interest of brevity.

It is known that such bands can be rendered more attractive by pigmentation, printing, dyeing, etc. (see U. S. A. Patents No. 1,997,769 to Fletcher, 2,071,024 to Clark, and 2,141,744 to Evans), as previously indicated, but up to the present time a band having a truly metallic appearance regardless of the use to which it is put,

has not been offered to the public or described in the literature. A demand for such a product has long existed, and much time and effort has been spent in research on this problem.

5 The production of a regenerated cellulosic band having the appearance of gold foil, was the primary object of this invention. Another object was to develop a non-fibrous band having clear and gold sections. Still other objects were 10 to improve the physical characteristics of shrinkable cellulosic bands, to produce cellulosic sheet material having a more metallic appearance than heretofore possible, and to produce by pigmenting and dyeing, cellulosic pellicles simulating thin metal sheet. A general advance in the art, and other objects which will appear hereinafter, 15 are also contemplated.

It has now been found that a cellulosic band having a metallic gold appearance can be prepared by dyeing a gel band having certain physical and chemical characteristics, with yellow sulfur dyes such as the thionation product of a mixture of meta-tolylene-diamine and benzidine. An outer layer (that which furnishes the 20 surface presented to the eye) containing about 45% thin, flat, ground mica particles, and an inner layer containing about 12% titanium dioxide pigment, these proportions being based on the cellulose present, provide the aforementioned 25 characteristic.

30 How the foregoing objects and related ends are accomplished will be apparent from the following exposition, in which are disclosed the principle and divers embodiments of the invention, including the best mode contemplated for carrying out the same. The written description is amplified by the accompanying drawing, in 35 which:

Figure 1 is an elevation view of a gel regenerated cellulose band of this invention;

40 Figure 2 is a perspective view of a section of tubing similar to that shown in Figure 1, but on a larger scale and with the parts broken away;

Figure 3 is a fragmentary perspective view of 45 the portion, indicated at J, of the band shown in Figure 2 but greatly enlarged to show the relation of the colored parts at their juncture;

Figure 4 is an end or plan view of a tube such 50 as that from which the flattened section shown in Figure 2 would be cut;

Figure 5 is a perspective view of a bottle top and its primary closure, having the gel secondary closure of Figure 1 in position for drying thereon;

Figure 6 is a perspective view of a bottle top

similar to that of Figure 5 but with the secondary closure in dried condition, sealing the primary closure and the bottle; and

Figures 7, 8 and 9 are diagrammatic views showing the relation of the viscose layers in the extrusion nozzles before they are joined to form the tube of Figure 4.

Referring now to the drawing, in which the relative dimensions have been considerably exaggerated for purposes of clarity in illustration, a gel regenerated cellulose band is indicated at 11 in Figures 1, 2 and 5, and a tube, of which said band would be a section, is shown at 1 in Figure 4.

The band in Figure 2 is shown with a part broken away, to better illustrate its construction. It has narrow, clear or transparent side portions indicated at 12, and opaque gold front and rear portions at 13. Inside the gold portions are opaque white portions 14.

In Figures 5 and 6, 28 indicates the neck of a bottle closed with a primary closure 21, and sealed with a revenue stamp 22. In conventional practice the transparent section 12 of the gel band is positioned over the revenue stamp, as shown in Figure 5, so that when the band dries the printing on the stamp is legible but completely covered and held tightly against the bottle neck, as shown in Figure 6.

The mechanical steps involved in producing these bands are generally conventional, being disclosed in U. S. A. Patent No. 2,141,776 to Vautier & Fays. They involve squirting concentric layers of viscose, contacting the squirted layers, and treating the resulting structure with a coagulating bath immediately after the layers are joined but before substantial diffusion of the different types of viscose can take place. One very satisfactory extruding scheme is illustrated in Figure 7, in which clear viscose layers are indicated at 72, opaque white layers at 74, and layers containing mica and yellow pigment, or equivalent coloring agent, at 73. Other acceptable arrangements are shown in Figures 8 and 9, wherein the numerals 82 and 84 indicate clear layers, 83 and 85 indicate the mica-containing layers, and 84 and 86 indicate the opaque titanium dioxide-containing layers.

Ordinarily the inner and outer layers are of equal thickness. Surface tension causes the finished bands to be in the same general arrangement, for example, that shown in Figure 4, whether or not the clear sections (72, 82 and 92) are equal or only half as thick as the opaque sections (73+74, 83+84 and 85+86).

The thickness of the gel band may be varied to suit individual requirements, but ordinarily a thickness of 0.017 inch, which gives a thickness of approximately 0.004 to 0.005 inch in the dry state, is employed. In all cases the white pigmented under layer must be thick enough to give opacity, for example 0.006 to 0.012, preferably 0.008 to 0.01 inch, and the outer mica layer must be thick enough to give, in cooperation with the other features, the desired metallic effect, preferably 0.008 to 0.01 inch.

Considerations of strength and shrinkage characteristics generally control the dimensions. Good results have been obtained when the titanium dioxide and mica-containing layers were not of the same thickness, but it is preferred that the thickness of each layer be within the range 30% to 70% of the total thickness of the band.

Preferably the outer layer contains 45% mica (based on the cellulose present), but satisfactory results can be obtained with proportions in the

range 30% to 60%. The amount of titanium dioxide contained in the opaque layer is 12% to 16%, preferably 12%, of the cellulosic material present in that layer.

5 Bands having a satisfactory gold appearance have been obtained by incorporating finely ground unreduced yellow vat dyes singly and in mixtures, within the mica layer. Preferably 1-(1':9' - isothiazolanthrone - 2' - carbonyl) - 6 - 10 chloro-anthraquinone and 1-(1':9' - isothiazolanthrone-2'-carbonyl) - amino-5-benzoyl-amino-15 anthraquinone are utilized for this purpose. The amount of the dye pigment so employed is preferably 6%, but acceptable results are obtained with 2% to 10% (based on the cellulose). Equal or superior gold appearances are obtained by dyeing the gel regenerated cellulose product with one or more yellow sulfur dyes. A particularly useful dye, for this purpose, is the 20 thionation product of a mixture of meta-toluylene-diamine and benzidine (see French Patent 321,183). The corresponding yellow sulfur dye from paratoluidine and benzidine (C. I. 955) is also quite satisfactory. A band may be both dyed and pigmented, if desired.

25 The present invention contemplates primarily a gold band, but it comprehends elements which can be advantageously applied with bands of other colors, for example, silver appearing bands, 30 superior to bands previously designed to simulate silver, may be produced by replacing the aforementioned yellow coloring matter with 0.1% to 0.5% of a black pigment such as colloidal graphite, carbon black, black vat dyes, and the like.

35 Preferably the size of the mica particles is within the range 20 to 150 microns (measured in the longest dimension), but this range is not absolutely critical and the size may extend somewhat both above and below this range. Wet 40 ground mica gives the most desirable results.

45 Preferably the size of the titanium dioxide pigment particles is within the range 0.5 to 2 microns average. Other white or light colored pigments may be used instead of, or in conjunction with, the titanium dioxide as the opaques in the under layer.

50 Instead of adding the color as a pigment to the viscose layer containing the mica, the tube, or the band after being cut therefrom, may be dyed in the conventional way. In such instances the clear window and the opaque layer will be colored.

55 The transparent section of the band may be omitted, if desired, in which case the tube would consist of uniform concentric layers, the outer of which contains the mica and yellow coloring matter, and the inner the titanium dioxide.

60 The bands may be formed of materials other than regenerated cellulose, for example, cellulose ethers and like materials, coagulable from aqueous or aqueous alkaline solutions. While the non-fibrous cellulosic pellicles are the most common type, in some instances pellicular bands formed of non-cellulosic materials such as gelatin, casein and the like, may be used.

65 The bands may be perforated to facilitate removal, as pointed out in U. S. A. patent application Serial No. 327,406, filed April 2, 1940, by Edwards & Mueller. Reference to that application is made for further details in this art.

70 There are numerous unexpected advantages in the present invention, for example, the strength of the gel band is 20% greater, and the strength of the dried band is 50% greater than a band consisting of a single layer having mica throughout. Improvements in shrinkage are also ob-

tained since the present band has 20% greater shrinkage.

As will be obvious from a consideration of the invention, the disadvantage of metal secondary closures which cannot provide a window, and heretofore known shrinkable closures which did not have a metallic look, are overcome. As a result, the bands have a wider appeal, since they furnish the esthetic effect demanded by customers, and the much desired utilitarian features such as transparent windows, tight fit, etc.

As many apparently widely different embodiments of this invention may be made without departing from the spirit and scope thereof, it is to be understood that this invention is not limited to the specific embodiments thereof except as defined in the appended claims.

We claim:

1. A shrinkable, cellulosic band secondary closure comprising essentially an outer metallic-appearance portion containing mica and coloring material and an underlying inner opaque portion containing a white pigment.

2. A shrinkable, cellulosic band secondary closure comprising essentially an outer metallic-appearing portion containing mica and coloring agent, and an underlying inner opaque portion containing titanium dioxide pigment.

3. A shrinkable, cellulosic band secondary closure comprising essentially an outer metallic-appearing portion containing 30%-60% mica and coloring substance, and an underlying inner opaque portion containing 12%-16% titanium dioxide pigment.

4. A shrinkable, cellulosic band secondary closure comprising essentially an outer metallic-appearance portion containing 30%-60% mica and yellow vat dye, and an underlying inner opaque portion containing 12%-16% titanium dioxide pigment.

5. A shrinkable, regenerated cellulose band secondary closure of gold appearance, comprising essentially an outer metallic-appearance portion containing about 45% mica particles within the range 20 to 150 microns (measured in the longest dimension) dyed with the yellow sulfur dye obtained by thionating a mixture of metatoluylene-diamine and benzidine, and an underlying inner opaque portion containing about 12% titanium dioxide pigment having a particle size of 0.5 to 2 microns.

6. A regenerated cellulose secondary band closure for bottles and the like, comprising a white pigmented section overlaid with a gold-appearing section containing mica and a yellow dye.

7. A regenerated cellulose secondary band closure for bottles and the like, comprising a white titanium dioxide pigmented section overlaid with a gold-appearing section containing mica and a yellow dye.

8. A regenerated cellulose secondary band closure for bottles and the like, comprising a white titanium dioxide pigmented section overlaid with a gold-appearing section containing 45% mica and a yellow dye.

RAYMOND E. T. HAFF.  
JOHN CONLYN CREADICK.  
THOMAS F. BANIGAN.